# EUROPEAN PATENT SPECIFICATION

(11) **EP 0 272 788 B1**
(45) Date of publication and mention of the grant of the patent: **01.07.1992**
(21) Application number: 87310035.8
(22) Date of filing: 13.11.1987
(51) Int. Cl.: C21D 5/00, C22C 37/00

(54) **A method of making wear resistant gray cast iron**
Verfahren zur Herstellung eines verschleissfesten Graugusseisens
Procédé de fabrication de fonte grise résistante à l'usure

(30) Priority: 22.12.1986 US 945145
(43) Date of publication of application: 29.06.1988
(73) Proprietor: FORD MOTOR COMPANY LIMITED, Brentwood, Essex CM13 3BW (GB); FORD FRANCE SOCIETE ANONYME, 92506 Rueil Malmaison Cedex (FR); FORD-WERKE AKTIENGESELLSCHAFT, 50725 Köln (DE)
(72) Inventor: Kovacs, Bela Victor, Bloomfield Hills Michigan 48013 (US)
(74) Representative: Messulam, Alec Moses

(56) References cited:
- EP-A- 0 018 703
- EP-A- 0 174 087
- FR-E- 89 010
- GB-A- 545 102
- GB-A- 840 490
- US-A- 3 384 515
- PATENT ABSTRACTS OF JAPAN, vol. 10, no. 71 (C-334)[2128], 20th March 1986; & JP-A-60 211 050 (TEIKOKU PISTON RING K.K.) 23-10-1985
- METAL PROGRESS, vol. 128, no. 2, July 1985, pages 19-26, Metals Park, Ohio, US; R.B. GUNDLACH et al.: "Austempered ductile iron combines strength with toughness and ductility"
- (2) METALS HANDBOOK, 9th Ed., Vol. 1, Properties and selection: Iron and Steels, p. 3-32.

## Description

The invention relates to a method of making wear resistant gray cast iron.

Grey cast iron is the least expensive of all the cast metals. This is due to the type of raw materials used; pig iron, cast iron scrap, steel scrap, limestone, coke and air, all of which are relatively inexpensive. Most gray cast iron used commercially is used primarily in the as-cast condition. There has been some attention to heat treatment and low alloying for grey cast irons through the years.

The general consensus of foundry operators in this country indicates that the composition of gray cast iron should be about (using weight percentages here and throughout the description); 2.0-4.0 carbon; 1.25-3.25 silicon; .75-1.25 manganese; .08-.12 sulfur; and .07-.20 phosphorus.

In the field of abrasive wear, gray cast iron is usually used where the required impact toughness in service is not severe. Such cast iron is resistant to abrasive wear because of the presence of a high amount of carbides in the matrix of the cast iron. Most gray cast irons will contain at least 10% by weight primary complex iron carbides. Unfortunately, however, these carbides are normally massive and impart a degree of brittleness to the cast iron which considerably limits its usefulness with reference to impact strength. While relegating gray cast iron to applications without the need for high impact strength, the main developmental effort has been to improve machining.

One attempt to provide greater machinability while retaining excellent wear resistance and fatigue resistance of gray cast irons involves heat treating the as-cast iron to reduce hardness while retaining the carbidic microstructure (see U.S. patent 4,230,506). In this patent, the cast metal was alloyed with a combination of carbide forming agents such as chromium, nickel, copper, molybdenum, and vanadium. They were used in combination to provide a composite total in an amount of 2.25-3.85%; this is a considerable amount of carbide forming agent. The improvement in machinability was achieved by heat treating to an austenitizing temperature, slowly cooling over a period of 1-1/2 hours to a temperature level of 400 F, and then air cooling. Slow cooling promoted the production of pearlite and reduced the hardness of such cast iron, making it more readily machinable. After machining, the iron was quenched to transform any retained austenite to martensite.

The problem with the 4,230,506 patent is that wear resistance is retained or improved at the sacrifice of toughness and strength characteristics, making it unsuitable for applications that require a high level for both of these characteristics.

Similarly, in U.S. patent 3,384,515, the solution to the problem of machinability was to control heat treating to permit the promotion of complex iron carbides while providing for incipient spheroidization of pearlite, thereby voiding martensite and reducing the hardness of the material. The same problem with respect to lack of enhancement of toughness and strength characteristics in such a carbidic cast iron remains.

In U.S. patent 2,885,284, an attempt was made to provide for an increase in both the abrasive wear as well as the impact properties of the gray cast iron. The contribution of this patent is to incorporate high amounts of alloying ingredients in the form of aluminium and manganese to promote contrary characteristics. Aluminium is added in amounts greater than 1% to promote graphitization and manganese is added in amounts greater than 1.5% to promote carbide stabilization. There is not attempt to modify or introduce any unusual heat treating parameters; there is simply a reliance upon conventional processing and heat treating steps. The disclosure admits, in column 2, lines 27-33, that the amount of aluminium or manganese that is incorporated will depend upon which characteristic is desired in the final product, namely, to increase toughness the carbon must be predominantly in the form graphite promoted by the use of aluminium, and to provide for increased hardness the carbon must be predominantly in the form of carbides, which is promoted by the incorporation of manganese. This disclosure is an "either/or" teaching in that the there is no suggestion that both of such characteristics can be achieved at a high level at the same time.

EP-A-0,174,087 discloses a method for making compacted graphite cast iron. A ferrous alloy is melted consisting of by weight 3-4% C, 2-3% Si, .2-.7% Mn, .25-.4 Mo, .5-3.0 Ni up to .002% sulphur, upto .02% phosphors impurities up to 1.0% and the remainder iron. The melt is subjected to graphite modifying agent to form compacted graphite upon solidification. The solidified casting is heat treated by austempering and quenching to produce an iron having matrix of bainite and austenite.

It is an object of this invention to provide a gray cast iron having both increased wear resistance and toughness which can be achieved by modification both in the chemistry and the heat treating techniques for gray cast iron.

In addition, it is an object of this invention to provide the above type of gray cast iron which additionally has high tensile strength, high damping capacity, high heat conductivity, and more ductility than conventional cast irons.

According to the present invention there is provided a method of making a wear resistant gray cast iron comprising, providing a hypoeutectic gray iron melt including by weight, 2.5-3.0% carbon, 2.0-2.5% silicon, .5-.9% manganese, and the reminder iron, solidifying said hypoeutectic gray iron melt to which has been added a carbide forming first agent in an amount of .3-.8% by weight, selected from the group consisting of titanium, vanadium, chromium and molybdenum, and a high carbon austenite-ferrite forming agents in an amount of .5-3.0%, selected from the group consisting of nickel and copper, said solidification being at a rate to form a matrix with a mixture of flake graphite and eutectic carbide suspended in said matrix, and heat treating said solid by (i) heating to a temperature and for a period of time to fully austenitize the solid, (ii) quenching said solid to a predetermined temperature level and holding at said level for a period of time to decompose austenite to form a high carbon austenite and ferrite matrix so that the carbon is present as 40-60% graphite and the remainder as eutectic carbide particles and (iii) air cooling the solid to room temperature.

Preferably, the heat treating comprises heating to a temperature level of 849-866 ° C (1560-1590 F) for a period of time of 1.5-2.5 hours; and the quenching step comprises quenching to a temperature level of 232-371 ° C (450-800 F) for a period of time of 1.5-2.5 hours. The rate at which such quenching is carried out is preferably in the range of 149-196 ° C (300-375 F) per minute.

The resultant cast iron will comprise a microstructure in which the carbon is present as 40-60% flake graphite and the remainder of the mixture eutectic carbide. Such mixture is controlled by the selection of the solidification rate and by the selection of chemistry for the gray cast iron melt. The casting will preferably have a tensile strength of 45-55 ksi (310-379 MPa), an impact strength of 30-35 ft/lb (2.05-2.4 m/N), and an elongation of about 2%. The wear resistance of such casting is 2-3 times greater than conventional gray cast irons and when measured by a standard sleeve test is .0028-.0019 inch per 1000 hours. The casting also is characterized by resistance to scuffing whereby the ratio of horsepower (power) to produce scuffing divided by the normal horsepower (power) is greater than 1.5. These wear resistance parameters are achieved through attainment of a type A graphite flake in the casting.

The invention will now be further described by way of example with referance to the accompanying drawings in which:
Figure 1 is a photo-micrograph of the structure of the casting produced by the method of this invention, the microstructure being shown at an enlargement of 500X. Areas of flake graphite, eutectic carbide, and austenite ferrite are indicated.

### Chemistry

A conventional wear resistant gray iron usually contains 3.0-4.0% carbon, 1.5-3.0% silicon, and .5-.9 manganese. The method of the present invention lowers the carbon content and adds both a carbide forming agent and an agent to facilitate the formation of high carbon austenite-ferrite during heat treatment. The carbide forming agent is made in addition to the normal carbide forming tendencies of manganese which is a normal part of gray cast iron. Aluminum is specifically absent from the present chemistry because it is a graphitizer which works against carbide formation and encourages pin hole defects. The addition of a graphitizing agent is conspicuously absent from the present invention because graphitization can be controlled through process parameters with a given lower amount of carbon.

Specifically, the chemistry comprises, preferably, 2.5-3.0% by weight carbon (a hypoeutectic iron- carbon alloy would comprise less than 4.35% carbon equivalent). If the carbon content were to be below 2.5%, it would be difficult to provide the desired amount of carbide/graphite ratio (40:60 to 60:40) that is necessary for the wear resistance of this invention. If the carbon content were in excess of 3%, processing parameters would tend to form an excessive amount of graphite. It is desirable for the starting melt for this invention that it have a carbon equivalent in the range of 3.2-4.35 because below 3.2 too much carbide is formed, and above 4.35 too much graphite is formed, making it difficult to control the graphite/carbide ratio. Silicon is present in an amount of 2.0-2.5% and manganese remains at .5-.9%. If the silicon and manganese contents were to be below the designated amounts of 2.0 and .5%, respectively, there would be insufficient volumes of graphite or carbide formation; if the upper limit of manganese was exceeded, Mn segregation will occur and a nonuniform matrix structure will result. If the upper limit of silicon is exceeded, excessive carbide and/or graphite formation will occur.

The additional carbide forming agent, which is added to the gray iron melt herein, comprises molybdenum, titanium, chromium, or vanadium. Any one or all of these ingredients may be added as long as they are present in the alloy melt in an amount in the range of .3-.8% as combined. If less than .3% is employed, the carbide volume will be too low; if greater than .8% is employed, then too much carbide will be present.

In order to promote the decomposition of austenite into high carbon austenite and ferrite, without the formation of pearlite or martensite, during the heat treatment and cooling sequence, it is desirable to add either nickel and/or copper in an amount of .5-3.0%, which functions as a pearlite suppressor and thus an austenite-ferrite former. If the amount of these elements, singly or combined, were to be below .5%, then pearlite formation in larger castings will occur, and if exceeding 3.0%, the alloying agent would be wasted and is uneconomical.

The above melt is fully solidified at a rate over a period of 4-16 minutes to ensure the formation of a carbon mixture in the form of 40-60% by volume graphite and the remainder eutectic carbide.

### Processing

The solidification of the melt as indicated above is then subjected to a heat treatment sequence which comprises heating to an austenitizing temperature in the range of 1560-1590 ° F (848.9-865.6 C) and held at such temperature for a period of 1.5-2.5 hours, during which time the casting will be fully austenitized. The casting is then quenched to a temperature level of 450-800 ° F (232-371 ° C) and held for a period of 1.5-2.5 hours. The quench rate should be in the range of 300-375 ° F (149-196 °C) per minute. If the quench rate were to be slower than 300 ° F (149 C) per minute, the opportunity for formation of pearlite would be increased. If the quench rate were to exceed 375 ° (196°C) per minute, the tendency for forming quenching cracks (due to high thermal stresses) would be experienced. The quench rate is important because it attempts, by way of processing, to determine the desirable matrix of austenite and ferrite. By observing the quench rate and the required chemistry, such heat treatment sequence will result in a cast iron matrix of austenite-ferrite having a suspended carbon mixture in the form of 40-60% flake graphite and the remainder in the form of eutectic carbide particles. This proportioned mixture is one of the key aspects of providing for simultaneous enhancement of wear resistance and impact resistance.

Following the decomposition of austenite to high carbon austenite and ferrite, the casting or solidification is then cooled to room temperature by air cooling.

### Microstructure

The resulting casting will have a microstructure which consists of a high carbon austenite and ferrite matrix with a suspended mixture of flake graphite and eutectic carbide particles. There is a conspicuous absence of martensite or pearlite in the microstructure. The suspended mixture particles constitute about 20% by volume of the microstructure. The graphite particles will be in the form of type A flake graphite because of good inoculation using ferro-silicon. Such type A graphite will influence the damping capacity, thermal conductivity, and machinability of the gray cast iron.

The physical characteristics of such gray cast iron will have a wear resistance which is at least 2-3 times greater than that of conventional gray cast irons, and with the limited samples that have been tested to date the wear resistance shows .0028-.0019 inch (0.07-0.048 mm) per 1000 hours of a conventional sleeve test, such test being outlined in the Metals Handbook.

In addition, the wear resistance is characterized by resistance to scuffing wherein the ratio of horsepower (power) to produce scuffing divided by the normal horsepower (power) is greater than 1.5. Gray cast iron, having a type A graphite in a martensitic matrix, normally exhibits a resistance to scuffing in the range of 1.39-1.45.

The impact resistance was tested to be in the range of 25-35 ft/lbs (1.7-2.4 m/N), where a conventional gray cast iron has a charpy notch impact value normally in the range of 1-2 ft/lbs (0.068-0.137 m/N).

The tensile strength of such resultant cast iron is 45-55 ksi (310-379 MPa), which is in the high range for gray cast iron, and elongation of about 1-2%. The hardness for such material is the range of 160-248 BHN.

### Examples

Several examples were prepared by melting a gray iron starting material which consisted of silicon in an amount of 2.3%, manganese .6%, with phosphorus being .12%, and sulphur being .10%. The carbon content of the gray iron was varied according to that shown in Table I along with variations in the added carbide forming agent, and variations in the addition of nickel as an agent to encourage the decomposition of austenite to high austenite and ferrite. Heat Treatment was employed as indicated (such treatment being to heat the casting to 1570° F (854 °C) for two hours, quench to 600 ° F (315 C), and hold for two hours, then air cool). The wear resistance and impact resistance were recorded for each such example.

## Claims

1. A method of making a wear resistant gray cast iron comprising, providing a hypoeutectic gray iron melt including by weight, 2.5-3.0% carbon, 2.0-2.5% silicon, .5-.9% manganese, and the reminder iron, solidifying said hypoeutectic gray iron melt to which has been added a carbide forming first agent in an amount of .3-.8% by weight, selected from the group consisting of titanium, vanadium, chromium and molybdenum, and a high carbon austenite-ferrite forming agent in an amount of .5-3.0%, selected from the group consisting of nickel and copper, said solidification being at a rate to form a matrix with a mixture of flake graphite and eutectic carbide suspended in said matrix, and heat treating said solid by (i) heating to a temperature and for a period of time to fully austenitize the solid, (ii) quenching said solid to a predetermined temperature level and holding at said level for a period of time to decompose austenite to form a high carbon austenite and ferrite matrix so that the carbon is present as 40-60% graphite and the remainder as eutectic carbide particles and (iii) air cooling the solid to room temperature.

2. A method as claimed in claim 1, in which said heating is carried out at 849-866 °C (1560-1590 °F) for 1.5-2.5 hours.

3. A method as claimed in claim 1 or 2, in which said quenching is carried out at 232-371 ° C (450-800 F) for 1.5-2.5 hours.

4. A method as claimed in Claim 3, in which said quench rate is 149-196 °C/minute (300-375 °F/minute).

## Revendications

1. Procédé pour produire une fonte grise résistant bien à l'usure, comprenant l'obtention d'une fonte grise hypoeutectique fondue comprenant, en poids, 2,5 à 3,0 % de carbone, 2,0 à 2,5 % de silicium , 0,5 à 0,9 % de manganèse, le reste étant du fer , la solidification de cette fonte grise hypoeutectique fondue à laquelle a été ajoutéé une quantité de 0,3 à 0,8 % en poids d'un premier agent formateur de carbure, choisi parmi le titane , le vanadium , le chrome et le molybdène , et une quantité de 0,5 à 3,0 % d'un agent formateur d'austénite-ferrite à forte teneur en carbone , choisi parmi le nickel et le cuivre , ladite solidification étant faite à une vitesse permettant de former une matrice comportant un mélange en paillettes de graphite et de carbure eutectique en suspension dans ladite matrice , et le traitement thermique dudit solide par (i) chauffage jusqu'à une température et pendant une période de temps permettant de rendre le solide entièrement austénitique ; (ii) refroidissement rapide dudit solide jusqu'à un niveau prédéterminé de température et maintien à ce niveau pendant une période de temps permettant de décomposer l'austénite pour former une matrice d'austénite et ferrité à haute teneur en carbone, de façon que le carbone soit présent sous forme de graphite à 40 - 60 % et le reste sous forme de particules de carbure eutectique , et (iii) refroidissement du solide à l'air jusqu'à la température ambiante

2. Procédé tel que revendiqué à la revendication 1 , dans lequel ledit chauffage est effectué à 849-866 ° C ( 1 560 - 1 590 ° F) pendant 1,5 à 2,5 heures .

3. Procédé tel que revendiqué à la revendication 1 ou 2 , dans laquel ledit refroidissement rapide est effectué à 232-371 ° C ( 450-800 ° F) pendant 1,5 à 2,5 heures .

4. Procédé tel que revendiqué à la revendication 3 , dans lequel ladite vitesse de refroidissement rapide est de 149-196 °C/minute (300 - 375 °F/ minute ) .

## Patentansprüche

1. Verfahren zur Herstellung von verschleißfestem Grauguß, das darin besteht, daß man eine hypoeutektische Graugußschmelze mit, gerichtsmäßig, 2,5 - 3,0% Kohlenstoff, 2,0 - 2,5% Silizium, 0,5 - 0,9% Mangan und dem Rest Eisen herstellt, jene hypoeutektische Graugußschmelze, die mit einem karbidbildenden, aus der Gruppe Titan, Vanadium, Chrom und Molybdän ausgewählten ersten Mittel in einer Menge von 0,3 - 0,8 Gew.-s% und einem kohlenstoffreichen austenit/ferrit-bildenden, aus der Gruppe Nickel und Kupfer ausgewählten Mittel in einer Menge von 0,5 - 3,0% versetzt worden ist, verfestigt, wobei diese Verfestigung derart erfolgt, daß eine Matrix mit einer Mischung aus Flockengraphit und in jener Matrix suspendiertem eutektischen Karbid gebildet wird, und diesen Feststoff tempert, indem man (i) auf eine zur vollständigen Austenitbildung des Feststoffes ausreichende Temperatur und über einen ausreichend langen Zeitraum erhitzt, (ii) jenen Feststoff auf eine vorbestimmte Temperaturhöhe abschreckt und auf dieser Höhe lange genug hält, damit der Austenit unter Bildung einer hochkohlenstoffhaltigen Austenit- und Ferritmatrix zersetzt wird, so daß der Kohlenstoff als 40 - 60% Graphit und der Rest als eutektische Karbidteilchen vorhanden ist, und (iii) den Feststoff auf Zimmertemperatur luftkühlt.

2. Verfahren nach Anspruch 1, worin jenes Erhitzen bei 849 - 866 °C (1560 - 1590°F) 1,5 - 2,5 Stunden lang er folgt.

3. Verfahren nach Anspruch 1 oder 2, worin jenes Abschrecken bei 232 - 371 °C (450 - 800 ° F) 1,5 - 2,5 Stunden lang erfolgt.

4. Verfahren nach Anspruch 3, worin jene Abschreckungsgeschwindigkeit 149 - 196°C/Minute (300 - 375 °F/Minute) beträgt.
